

June 19, 1945.

W. DAWIHL

2,378,539

PROCESS OF MAKING SHAPED BODIES CAPABLE OF BEING SINTERED

Filed Sept. 4, 1941



Inventor:  
Walther Dawihi,  
by Harry E. Schubauer  
His Attorney.

## UNITED STATES PATENT OFFICE

2,378,539

PROCESS OF MAKING SHAPED BODIES  
CAPABLE OF BEING SINTEREDWalther Dawihl, Kohlhasenbrück, near Berlin,  
Germany; vested in the Allen Property Custo-  
dianApplication September 4, 1941, Serial No. 409,501  
In Germany June 4, 1940

3 Claims. (Cl. 18—55)

Shaped bodies particularly of the kind made of hard metal alloys have heretofore usually been produced in such a way that a powder, for instance a mixture of powdered tungsten carbide and powdered cobalt, was placed into molds either in the dry state or with an addition of a moistening liquid, such as water or acetone, and subsequently pressed, after which a greater number of the small pressed-powder bodies thus obtained were sintered conjointly in a furnace and then, after being machined, again placed in a furnace in order to be finish-sintered.

The object of the invention is to provide a considerable reduction in time, and consequently an increase in economy, of the production process of said shaped bodies capable of being sintered. This is achieved if the pressing operation is effected by means of extrusion presses suitably designed. The powder, which has been moistened with a suitable binder, is accordingly charged into an extrusion press, in which the forward movement of the mass is interrupted at short regular intervals in order that a portion of the mass, while retained in the press during its stand-still, can first be de-aerated and then suddenly set under an air or gas pressure, if necessary, of several atmospheres. Each section of the forward movement of the flowing mass corresponds in length to the section of the mass that is being acted upon by vacuum, air or gas. Therefore, the bar extruded from the mouth-piece of the press has been uniformly subjected over its entire length to the action of the vacuum, air or gas. Furthermore, the extruded bar is divided in manner known per se into sections of the required length. Such sections are subsequently sintered, machined to the desired shape, and finish-sintered. As a binder, use can be made of water, organic liquids, such as for instance glycerine or mixtures containing glycerine, or also solutions, for instance, of resins in the liquids just referred to. In consequence of de-aeration, the air trapped in the pores of the hard metal mass is first exhausted and then, owing to the sudden stream of gas entering under sufficient pressure, the total mass is compressed, and the cavities which were filled with the vapour from the moistening liquid during the de-aeration, are compressed to a large extent and closed, thus liquefying such evaporated parts. The gas used can either be air or, in the case of powders sensitive to oxygen, hydrogen or other gases. In general, the pressure of the gas introduced will be adjusted to one atmosphere; however, in certain cases, pressures of several atmospheres may also be adopted. Owing to

its plasticity the extruded bar can readily be sectioned by customary means, such as knives or cutting wires. It is possible by means of the novel method to produce per hour many hundreds of units of shaped bodies of uniform size, measuring for instance 10 by 10 by 20 mm. along the edges, such as are frequently used as blanks for cutting-tips insert-pieces and pins.

In order that the invention may be readily understood, one example of construction of an extrusion press suitable for carrying out the process is represented diagrammatically on the accompanying drawing showing a vertical section.

The extrusion press consists of a cylindrical casing 1 having a tapered front portion, and which encloses a longitudinally arranged shaft 2 as well as a worm gear 3 secured thereto. At the rear end of the casing 1, a feed hopper 4 is provided for the powder which is mixed with a binder, for instance water or glycerine. Said hopper may contain, as shown, a piston 5, the action of which presses the powder 6 into the casing 1, avoiding the inclusion of an unduly great amount of air. The central portion of the casing 1 is separated from the rear and front parts of the casing by means of two screen plates 8 inserted therein and secured to bushings 7 of the shaft 2. To the wall of said central portion is fitted a tube 9 communicating, on the one side, with a pressure chamber by means of a shut-off valve 10 and, on the other side, with a vacuum source by means of a shut-off valve 11, so that either the air contained in the space between the two screen plates 8 can be exhausted or the space itself set under pressure. In this case, layers of the moist pasty powder-mixture, adhering to the screen plates 8, form a sufficiently tight air seal in the central portion of the casing, so that the action of the vacuum or of the pressure, as the case may be, can only become effective in the said central portion of the casing. In the mouth-piece 12 of the extrusion press is inserted a spring sleeve 13, the rear part 14 of which is attached to the inner wall of the mouth-piece 12, for instance by soldering, welding, or riveting. The front end of the sleeve 13 is subjected to the pressure exerted by a lubricating liquid, such as water or oil, introduced into the mouth-piece by means of two tubes 15. At the front end of the sleeve 13, the lubricating liquid is projected onto the bar, preventing the latter from adhering to the inner wall of the mouth-piece, which is an important feature in view of the risk involved for the bar to stick to the mouth-piece during each interruption of the forward movement of the bar. However, the lu-

bricating liquid which is continuously fed onto the surface of the bar, through the medium of the spring sleeve 13, causes the bar to be extruded very reliably in a constantly uniform condition from the mouth-piece 12. Directly in front of said mouth-piece, cutting tools of any desired description may be arranged to cut the bar into small shaped bodies. If desired, the piston 5 may be inserted with a perfectly tight fit to permit of the press chamber being set under vacuum or pressure as far as the said piston. With this arrangement, the first of the two screen plates may be dispensed with.

What I claim as new and desire to secure by Letters Patent of the United States is:

1. The process of making shaped forms of sinterable powder mixtures of hard metal alloys and the like which comprises intermittently advancing the powdered mixtures longitudinally through a press having three successive zones divided by transverse screens, interrupting the advance of the material at short intervals and during said interruption subjecting the material in the intermediate zone between the screens to de-aeration by vacuum, subjecting the material to superatmospheric gas pressure and finally extruding the treated material.

5 2. The process of making shaped forms of sinterable powder mixtures of hard metal alloys and the like and a liquid binder, which comprises intermittently advancing the powdered mixtures longitudinally through a press having three successive zones divided by transverse screens, interrupting the advance of the material at short intervals and during said interruption subjecting the material in the intermediate zone between the screens to de-aeration by vacuum, subjecting the material to superatmospheric gas pressure and finally extruding the treated material.

10 3. The process of making shaped forms of sinterable powder mixtures of hard metal alloys and the like and a liquid binder, which comprises intermittently advancing the moistened powder mixture longitudinally through a press having three successive zones divided by transverse screens, interrupting the advance of the material so that each successive portion will pause in the intermediate zone between the screens, subjecting such portion to de-aeration by vacuum and subsequently to superatmospheric gas pressure, advancing the material and finally extruding said 15 treated material.

WALTHER DAWIHL.